

**1**

3,824,078

**ALKALI SOLUBLE RAYON TEXTILE MATERIAL  
AND PROCESS FOR PRODUCING SAME**

Daniel J. Egan, New Foundland, N.J., assignor to Londat  
Aetz Fabric Co., Elizabeth, N.J.  
No Drawing. Filed Nov. 8, 1971, Ser. No. 196,780  
Int. Cl. D06m 11/02

U.S. Cl. 8—120

8 Claims

**ABSTRACT OF THE DISCLOSURE**

Alkali soluble textile materials produced without resorting to a carboxymethylation step by the impregnation of rayon with an aqueous solution of chromic acid or periodic acid, the resultant material being highly soluble in alkaline dissolving baths, such solution being free of gummy residues.

**BACKGROUND OF THE INVENTION**

In Pat. No. 2,921,934, issued Jan. 19, 1960 there is disclosed a procedure for converting cotton textile materials to alkaline soluble form by initially treating the cotton with suitable reagents to convert the same to carboxymethyl cellulose. The carboxymethylcellulose is then impregnated with a solution of chromic acid or periodic acid. The resultant acid treated material shows good solubility in alkaline dissolving baths and is free of gummy residues which are highly undesirable, particularly when the acid treated material is used as a backing for making lace, or in other textile products.

However, the preliminary treatment of the cotton fabric or thread to convert the same to carboxymethyl cellulose represents a substantial cost factor in the finished material; taking into account the cost of the necessary chemicals and the increased labor, time and equipment required for the initial conversion step.

Accordingly, an object of this invention is to provide an improved process for making alkaline soluble textile materials, wherein rayon fabric or threads are directly treated with an aqueous solution of chromic acid or periodic acid; the acid treated material being highly soluble in alkaline dissolving baths and free from undesirable gummy residues.

Another object of this invention is to provide a process of the character described wherein rayon fabrics of fine texture are converted to alkaline soluble form; such converted fabrics retaining substantially their original texture and strength thereby facilitating lace making operations wherein the converted fabric provides backing means in the lace making procedure.

Another object of this invention is to provide an improved alkaline soluble fabric derived from rayon of selected textures and qualities, with minimal manufacturing costs of the same by reason of the simplified chemical treating procedures involved; the treated fabric retaining substantially its original texture and strength so as to be particularly useful in the art of lace making.

Still another object of this invention is to provide an improved chemical treating procedure to rayon, whether made by the cuprammonium, xanthate or saponified cellulose acetate process, to produce a material which is highly soluble in alkaline dissolving baths; the acid of the treating procedure leaving the original physical form of the rayon unchanged with a retention of a substantial portion of the tensile strength of the untreated rayon.

Other objects of this invention will in part be obvious and in part hereinafter pointed out.

**DESCRIPTION OF THE PREFERRED  
EMBODIMENTS**

It has been found that rayon fabrics of varying textures may be readily converted to an alkaline soluble form,

**2**

by direct treatment or impregnation of the fabric with chromic acid or periodic acid. Upon correlating acid concentrations, temperatures and impregnation intervals, the acid treated fabric will retain substantially its original strength and texture. Further such acid treated fabrics will be highly soluble in alkaline dissolving baths such as aqueous solutions of sodium hydroxide or the like.

The following examples illustrate the invention:

**Example 1**

10 A woven Bemberg rayon fabric of a 76 x 76 thread count, was soaked for 90 seconds at 75° C. in an aqueous impregnating solution containing by weight 3% sodium bichromate and 4% concentrated sulfuric acid.

15 The acid treated fabric was then removed from the impregnating solution and washed with water. The washed fabric was dried and showed substantially the tensile strength and texture of the original fabric. The acid treated fabric was then placed in a boiling 10% aqueous solution of sodium hydroxide, by weight. The acid treated fabric dissolved rapidly. On filtering and weighing a small non-gummy residue, the solubility of the converted fabric in the sodium hydroxide solution was calculated as 99.4%.

20 The foregoing procedure was repeated except that the Bemberg rayon fabric was replaced by a viscose rayon fabric. The acid treated material showed a high solubility in a sodium hydroxide bath and no gummy residue.

**Example 2**

25 Bright, non-pigmented rayon yarn derived from saponified cellulose acetate, was soaked in a 4% aqueous solution of chromic acid, by weight, for 90 seconds at 75° C. The acid treated yarn was then washed and dried. On placing the acid treated yarn in a boiling bath of 9% aqueous sodium hydroxide, by weight, the same showed a solubility of 98.9% and with no gummy residue. The acid treated yarn retained substantially the tensile strength of the original, untreated yarns.

**Example 3**

30 A woven viscose rayon fabric of an 80 x 70 thread count, was soaked for 90 seconds at 75° C. in a solution of 4% sulfuric acid and 3% periodic acid by weight. After washing and drying the acid treated fabric, the same was dissolved in a 8% aqueous solution of sodium hydroxide, showing a solubility of 97.9%. The acid treated fabric retained substantially its original texture and tensile strength.

**Example 4**

35 40 A woven viscose rayon fabric of a 48 x 40 thread count, was soaked for 90 seconds in a 4% aqueous solution of chromic acid at 85° C. The acid treated fabric retained its original form after washing and drying.

45 The acid treated fabric was then placed in an 8% aqueous solution of sodium hydroxide at 35° C., for a half hour. Solution of the fabric took place to the extent of 98.4%.

**Example 5**

50 55 The procedure set forth in Example 1 was repeated except that the temperature of the sulfuric acid-sodium bichromate solution was 40° C. The impregnating time was extended to 10 minutes. The acid treated fabric was then washed and dried. The fabric was then dissolved in 10% sodium hydroxide, by weight, showing a solubility of 97.4% without a gummy residue. The acid treated fabric retained substantially its original texture.

**Example 6**

60 65 A viscous rayon fabric was treated with 15 seconds with an aqueous solution containing by weight 10% concentrated sulfuric acid and 4% sodium bichromate, at 90° C. The acid treated fabric was then washed and dried

and then placed in a 10% aqueous solution of sodium hydroxide at 90° C. The fabric dissolved to the extent of 98.7%.

**Example 7**

A Bemberg rayon fabric was treated for 90 seconds with an aqueous solution of 9% concentrated sulfuric acid and 4% sodium bichromate, at 75° C. The acid treated fabric was washed and dried, showing the original texture and substantially the strength of the original fabric. The treated fabric was then placed in an 8% aqueous solution of sodium hydroxide at 30° C. for ½ hour. Solubility was 97.8% and there was no gummy residue.

**Example 8**

A cuprammonium rayon fabric was soaked for 5 seconds in an aqueous solution containing by weight 6% sodium bichromate and 12% concentrated sulfuric acid. The soaking took place at a temperature of 75° C. The acid treated fabric was then washed and dried and then treated with a 10% aqueous solution of sodium hydroxide at the boil. The treated fabric dissolved to the extent of 98.9%.

The chromic acid or periodic acid treatment of the rayon, in fabric, yarn or nonwoven form, may be based on aqueous solutions of such acids or combinations of reagents forming the acid in situ. The acid treatment may be effected at temperatures ranging from room temperature to boiling and with acid concentrations varying by weight, from 0.5% to 50%. A preferred range of acid concentrations is between 4% and 10%.

With higher acid concentrations, impregnation interval is reduced and may be as little as a few seconds. The treating temperature is adjusted in inverse relation to acid concentration. Also, with relatively low acid concentrations, the impregnation period is extended and may range up to 20 hours.

It is understood that the acid treated fabric is washed with water in suitable washing tanks and dried with equipment known in the art.

In all cases, the conditions of acid treatment of the selected rayon fabric, yarn or thread, with chromic acid or periodic acid, is such as to leave the original physical form of the untreated fabric. Thus, the tensile strength of the treated fabric is substantially that of the original fabric. Such acid treated fabric may be readily handled in reeling machines and lace making machines, as well as other textile equipment, as may be used in the manufacture of lace on an alkaline solubilized backing.

The acid treated rayon in yarn form, may be incorporated in textile fabrics including conventional textile yarns which are not readily soluble in alkaline solutions. The finished fabric is then treated in an alkaline bath dissolving the alkaline soluble yarns, to thereby produce selected textile affects.

The term Rayon as used herein refers to regenerated cellulose having a lower degree of polymerization than that of natural cellulose such as cotton, wood pulp and the like. Further such terminal includes rayon produced by the xanthate process (viscose); cuprammonium (Bemberg) and by saponification of cellulose acetate.

The acid treated rayon of the instant invention may be dissolved in alkaline solutions of a wide range of concentrations, being soluble in aqueous solutions of sodium hydroxide having a concentration of from about 0.1% to about 35.0%. It is understood that in lieu of sodium hydroxide, other alkaline reagents may be used, including potassium hydroxide, lithium hydroxide, sodium carbonate, trisodium phosphate and the like.

I claim:

1. The process of forming alkali soluble textile material without resorting to a carboxymethylation step which comprises impregnating rayon with an aqueous solution of an acid selected from the group consisting of chromic acid and periodic acid under concentration, time and temperature conditions sufficient to obtain a modified textile material which retains the physical form and a major portion of the strength of the untreated rayon and which is highly soluble in alkaline dissolving baths and free of gummy residues as an incident to the solution thereof in said baths.
2. The process of Claim 1 wherein said acid is chromic acid.
3. The process of claim 2 wherein said acid has a concentration of from 0.5% to 50.0%.
4. The process of Claim 3 wherein the time and temperature of the acid impregnation is inversely related to the acid concentration.
5. Textile material produced by the process of Claim 1.
6. The process of Claim 1 wherein said rayon is viscose rayon.
7. The process of Claim 1 wherein said rayon is cuprammonium rayon.
8. The process of Claim 1 wherein said rayon is saponified cellulose acetate.

**References Cited**

**UNITED STATES PATENTS**

- |    |           |        |                  |       |         |
|----|-----------|--------|------------------|-------|---------|
| 45 | 2,921,934 | 1/1960 | Weisberg         | ----- | 8—129 X |
|    | 3,493,319 | 2/1970 | Berni et al.     | ----- | 8—120   |
|    | 3,385,653 | 5/1968 | Whitfield et al. | ----- | 8—120 X |
|    | 2,938,765 | 5/1960 | Reinhardt et al. | ----- | 8—120 X |

50 RICHARD D. LOVERING, Primary Examiner

U.S. CL. X.R.

260—212